

## UNITED STATES PATENT OFFICE

ALAN RICHARD POWELL AND ARTHUR WILLIAM SCOTT, OF LONDON, ENGLAND, AS  
SIGNORS TO JOHNSON-MATTHEY & COMPANY LIMITED, OF LONDON, ENGLAND

## ELECTRODEPOSITION OF PLATINUM

No Drawing. Application filed January 22, 1932, Serial No. 588,235, and in Great Britain March 12, 1931.

This invention relates to the electrolytic deposition of platinum from aqueous solutions and to the preparation of suitable plating salts for this purpose.

5 It has already been proposed to deposit platinum electrolytically as a bright plate from baths consisting of a solution of platinum hydroxide (hexahydroxyplatinic acid) in caustic alkalies. This type of bath usually contains about 4 per cent of free alkali metal hydroxide and is operated at temperatures below 35° centigrade with a current supplied at 2 volts. Although a bath prepared in this manner may yield good bright 10 deposits for some time after being freshly made up, it rapidly becomes turbid and a deposit of hydrated platinum trioxide forms on the anode; with more prolonged use a heavy flocculent precipitate of various platinum compounds is formed, whereby the effective 15 platinum content of the bath is reduced and the deposits become dull, patchy and loosely adherent.

It has also been proposed to employ neutral 20 solutions containing potassium platinate and magnesium borocitrate as baths for plating purposes, but these baths have found no commercial application. If these baths are rendered even slightly alkaline a grey flocculent 25 deposit of metallic platinum is produced.

The present invention has for its principal object to overcome these difficulties and to provide stable baths from which bright platinum deposits may be obtained of almost any 30 desired thickness.

According to this invention we utilize an alkali metal platinate bath to which is added a stabilizer and which is then rendered almost neutral by the addition of a mineral 35 acid. This bath gives no deposit of platinum on the cathode when operated at temperatures below 40° centigrade, but at higher temperatures especially above about 65° centigrade a brilliant, white, smooth and firmly adherent deposit is obtained.

As a stabilizer we prefer to use substances which form soluble complexes with platinum, such, for example, as oxalic, phosphoric or nitrous acids, or salts thereof. We have obtained particularly good results by the use of

an alkali metal oxalate, as for example sodium oxalate which prevents the formation of platinum trioxide, or compounds thereof on the anode, and retards or prevents the development of a flocculent precipitate in the bath, 55 thus rendering it stable over long periods.

In order to obtain good results with this bath we have found it necessary to keep the free alkalinity corresponding with a sodium hydroxide content of less than 2.5 per cent 60 and advantageously between 0.2 and 1 per cent. As the platinum is removed from the electrolyte by plating, the free alkalinity of the bath will increase and consequently it is necessary to keep this increase within the limits just mentioned by occasional neutralization of the liberated sodium hydroxide by the addition of sulphuric acid; this is most conveniently effected when the bath requires replenishment with platinum as hereinafter described. 65 70 75

The following examples illustrate methods of preparing plating baths according to this invention but the invention is not restricted to these examples.

## Example 1

100 ounces of sodium chloroplatinate ( $\text{Na}_2\text{PtCl}_6 \cdot 6\text{H}_2\text{O}$ ) are dissolved in 6 gallons of hot water and 100 ounces of sodium hydroxide in solid form are then added to the hot solution. The liquid boils vigorously so that cold water must be added as required to keep the boiling under control. When all the sodium hydroxide has been added, the 80 solution is diluted to 12 gallons with hot water and boiling is continued for from 3 to 4 hours until the colour of the liquid changes from orange to pale yellow; when the liquid has cooled slightly, a solution of 16 ounces of oxalic acid is added to form 17 ounces of sodium oxalate in the mixture and this is followed by 37 ounces of sulphuric acid diluted with water. The platinum solution will now contain 17 ounces of free sodium hydroxide 90 and after dilution to 24 gallons it contains approximately 1 per cent of platinum and 0.5 per cent of free sodium hydroxide. The sodium chloride, formed by the reaction of the sodium hydroxide with the sodium chlo- 95 100

roplatinate and the sodium sulphate, formed by the subsequent partial neutralization with sulphuric acid, act as conducting salts and increase the conductivity and throwing power 5 of the plating bath.

*Example 2*

If an excess of sulphuric acid be added to the solution resulting from the reaction of 10 the sodium hydroxide with the sodium chloroplatinate, a precipitate of hydrated platinic oxide ( $\text{PtO}_2 \cdot 4\text{H}_2\text{O}$ ) is obtained; this precipitate may be washed free from soluble salts and dissolved in sodium hydroxide solution 15 to yield an alkali metal platinic solution from which a plating bath may be prepared according to this invention by adding sufficient sodium hydroxide to give a free alkalinity of less than 2.5 per cent and preferably of from 0.2 to 1.0 per cent, the requisite 20 quantity of sodium oxalate, for example 0.5 per cent and sufficient sodium sulphate, for example 3 per cent to give a good throwing power. 25

In the aforesaid examples any other alkali metal hydroxide may be used in place of sodium hydroxide and any other soluble compound of tetravalent platinum, except cyanide complexes, may be used in place of the 30 sodium hexahydroxyplatinate.

These baths are operated above 40° centigrade and preferably at 65° to 85° centigrade with a current density of up to 20 amperes per square foot at 1.5 volts or higher; there 35 is no evolution of hydrogen at the cathode and the current efficiency is practically 100 per cent. Bright adherent deposits of platinum are obtained with these baths on polished gold, silver, copper, brass, bronze and 40 nickel-silver surfaces, but nickel, iron and steel surfaces must first be coated with copper and/or silver from an alkali metal cyanide bath.

Satisfactory plates are produced until the 45 platinum content of the bath falls to about 0.4 per cent; replenishment of the bath with platinum is then effected by adding the requisite quantity of platinic hydroxide prepared as hereinbefore described. This may 50 be added as a wet sludge, but is preferably previously dissolved in the minimum quantity of alkali metal hydroxide solution. In the latter case sulphuric acid equivalent to 55 this alkali metal hydroxide must be added to the plating bath after the replenishing solution has been added so as to maintain the alkalinity at approximately constant value.

What we claim is:—

60 1. A process for the electrodeposition of platinum in the form of a bright plate in which the electrolyte comprises a solution containing an alkali metal platinic, a conducting salt, a stabilizing salt and an alkali 65 metal hydroxide in an amount equivalent to

less than 2.5 per cent of free sodium hydroxide.

2. In the process as claimed in claim 1 employing as the stabilizing salt an alkali metal oxalate, preferably sodium oxalate. 70

3. In the process as claimed in claim 1 maintaining the free alkalinity at the equivalent of 0.2 to 1 per cent of sodium hydroxide.

4. In the process as claimed in claim 1 operating the bath at a temperature above 40° 75 centigrade and preferably at 65° to 85° centigrade.

5. In the process as claimed in claim 1 replenishing the bath by the addition of a solution of hydrated platinic oxide in an alkaline 80 solution.

6. In the process as claimed in claim 1 controlling the alkalinity within the limit specified in claim 1 by the occasional addition of an acid and preferably sulphuric acid. 85

7. In the process as claimed in claim 1, controlling the alkalinity at the equivalent of 0.2 to 1% of sodium hydroxide by the occasional addition of an acid and preferably sulphuric acid. 90

In testimony, we have signed our names to this specification at, London, England, this 4th day of January, 1932.

ALAN RICHARD POWELL.  
ARTHUR WILLIAM SCOTT.

95

100

105

110

115

120

125

130